

## UNITED STATES PATENT OFFICE

EARL H. BUNCE AND GEORGE T. MAHLER, OF PALMERTON, PENNSYLVANIA, ASSIGNEES TO THE NEW JERSEY ZINC COMPANY, OF NEW YORK, N. Y., A CORPORATION OF NEW JERSEY

## REDUCING ZINCIFEROUS MATERIALS

No Drawing.

Application filed January 4, 1928. Serial No. 244,401.

This invention relates to the reduction or smelting of zinciferous materials containing other contaminating metals whose boiling temperatures are above that of zinc but which accompany the gaseous product of the zinc smelting operation. The invention aims to provide certain improvements in the smelting of such zinciferous materials whereby an effective elimination of such other contaminating metals is obtained.

Lead, tin, antimony, bismuth, aluminum and magnesium are commonly present in zinc ores and their concentrates. While these metals, and perhaps others less well-known but commonly found in zinc ores such as germanium and thallium, boil at temperatures above the boiling temperature of zinc, nevertheless appreciable amounts thereof find their way into the gaseous product of the zinc smelting operation and thereby contaminate the zinc product obtained therefrom. Lead is one of the most common contaminants of zinc ores and their concentrates, and when present in relatively small amounts prevents the production by pyrometallurgical methods of high grade zinc products, such as zinc metal, zinc oxide, zinc dust, etc., substantially free of lead. A relatively large tonnage of zinc concentrates containing from 0.05 to 5% of lead are available for zinc smelting, but no entirely satisfactory pyrometallurgical method has heretofore existed for producing substantially lead-free zinc products therefrom. Similarly, tin, antimony, bismuth, germanium and probably thallium, aluminum and magnesium when present in the zinc smelting charge, will, to some extent at least, contaminate the zinc product obtained from the smelting operation, and while such contaminating metals are ordinarily present in relatively small percentages, frequently amounting to mere traces, they very often deleteriously influence the properties of the ultimate zinc product.

The object of our present invention is to provide a pyrometallurgical treatment for zinciferous materials containing one or more of the aforementioned contaminating metals in the course of which a substantial removal of the contaminating metals is effected, there-

by making possible the recovery of a purer and more desirable zinc product than can be obtained by the heretofore customary methods of zinc smelting. Since, in the practice of the invention, all of the contaminating metals appear to behave similarly, we will herein more particularly describe the invention with respect to the elimination of lead. The invention may be practiced solely for the elimination of lead without special regard to the elimination of other metals, or it may be practiced for the elimination of any one or more of the contaminating metals. In general, the elimination of substantially all of the lead by the practice of the invention will at the same time effect a substantial elimination of such others of the contaminating metals as may be present in the zinc smelting charge. Throughout the specification and the appended claims, we intend the terms "contaminating metals" and more particularly "lead" to include both the metallic form of these metals and compounds thereof. On the other hand, such lead-content figures as are given in the specification are percentages of lead calculated as metallic lead.

The present invention is based on our discovery that under appropriate conditions lead can be almost completely removed from the gaseous product of the zinc smelting operation by passing the gaseous product through a body of appropriate aggregates maintained at an appropriate elevated temperature in a reducing environment. We have also discovered that other metals whose boiling temperatures are above that of zinc but which accompany the gaseous product of the zinc smelting operation can be similarly removed, in large part at least, from the gaseous product. We have found that the aggregates may be any material which will withstand the prevailing temperature and not react with zinc so as to affect its subsequent recovery by condensation or otherwise. While the principles of these discoveries appear to be of general application, we have found that practical considerations make it desirable that the gaseous product be supplied in a substantially continuous stream of practically constant volume and composi-

tion and relatively free of oxidizing gases.

Based on these discoveries, our present invention involves smelting zinciferous material containing one or more contaminating metals so as to produce a substantially continuous stream of the resulting gaseous product, preferably of relatively constant volume and composition and practically free of oxidizing gases, and conducting this substantially continuous stream of the gaseous product through an appropriate eliminating medium maintained under reducing conditions at an elevated temperature but sufficiently low to effect substantial removal of the contaminating metal or metals from the gaseous product. The gaseous product, thus substantially freed of lead, and/or other contaminating metals, passes on to the subsequent treatment operation for the recovery of its zinc content. The eliminating medium is appropriately confined and arranged intermediate the zinc smelting chamber and the zinc recovery apparatus so that the gaseous product of the smelting operation passes in a substantially continuous stream from the reducing chamber through the eliminating medium to the zinc recovery apparatus.

The eliminating medium may be composed of any material which will withstand the prevailing temperature and not react with or contaminate the metallic zinc vapor so as to affect the subsequent condensation of the zinc vapor or the subsequent recovery of the zinc in other forms than zinc metal. Thus, the eliminating medium may be composed of graphite, coke, or other suitable carbonaceous material, clay refractories, silica refractories, alumina refractories, silicon carbide, partially crushed zinc ore, and the like. The zinc smelting charge itself consisting of a mixture of zinciferous material and carbonaceous reducing agent, preferably briquetted or otherwise agglomerated, is admirably adapted as the eliminating medium.

The eliminating medium should provide a multiplicity of tortuous paths for the flow therethrough of the gaseous product and should yet be sufficiently porous to permit the free passage of the gaseous product. These conditions are satisfactorily attained when the eliminating medium is composed of a body of aggregates. The aggregates may be naturally formed such as crushed or broken coal, ore and the like, or may be artificially formed such as briquettes, sinter, crushed or broken refractories and the like. The aggregates should be approximately uniform in size in order that the porosity of the eliminating medium as a whole may be substantially uniform. Furthermore, in order to provide the desired multiplicity of tortuous gas passages, the aggregates should not be too large. We have secured very satisfactory results with an eliminating medium composed of briquettes approximately three

inches in diameter or thickness confined in a vertically disposed cylinder about 15 inches internal diameter and about 6 feet long or high, where approximately one ton of zinc metal was recovered each 24 hours from the gaseous product passing through the eliminating medium.

It is our belief that the removal of lead, and other contaminating metals, by the eliminating medium is most effective, and probably only possible, when the lead is present in the metallic state. The eliminating medium must therefore be maintained under reducing conditions or in a reducing atmosphere free of any oxidizing influence, in order to inhibit the oxidation of metallic lead and zinc, and, if necessary, to reduce any oxidized lead or zinc that might be present in the gaseous product. Should air or other oxidizing gas leak into or otherwise enter the enclosure for the eliminating medium, the effectiveness of the lead removal is seriously impaired, if not completely destroyed. Preferably, the smelting operation is conducted so that the gaseous product thereof consists mainly of carbon monoxide and metallic zinc vapor with only a fraction of a percent of carbon dioxide. Where the carbon dioxide content of the gaseous product of the smelting operation exceeds about 1 to 2%, the eliminating medium should be composed of or contain a material capable at the prevailing elevated temperature of reducing carbon dioxide, such, for example, as coal, coke, charcoal or other carbonaceous material, in order to insure the necessary reducing conditions for effective lead removal.

While we are not now prepared to offer any positive theory of what actually takes place in the eliminating medium in the course of the practice of the invention, we will state what we now consider the most acceptable explanation of the phenomena underlying the invention, since this explanation furnishes plausible reasons for the necessity of observing the precautions and conditions herein described. The contaminating metals are present in the zinciferous material as compounds of the metals, such, for example, as oxides, sulfides, or the like. Certain of these metal compounds, for example, lead oxide and lead sulfide, volatilize readily at the temperatures prevailing in the zinc smelting charge, although the boiling temperatures of the metals themselves are considerably higher. These volatilized metal compounds are in contact with carbon monoxide in the smelting chamber and are thereby reduced and form minute metal particles which accompany the gaseous product of the smelting operation. Or it may be that the metal compounds are directly reduced without first volatilizing. Unless thus reduced to the metallic state, these readily volatile metal compounds will remain with the gaseous

product and not be removed therefrom in the passage through the eliminating medium; hence the necessity of maintaining the eliminating medium under reducing conditions.

- 5 The reduced contaminating metals are probably present in the gaseous product as very minute molten metal particles or droplets resembling a mist. In passing through the multiplicity of tortuous gas passages 10 provided by the eliminating medium these minute metal particles are thrown against the surfaces of the medium and probably caused to coalesce to some extent thereby forming larger particles less readily carried along 15 by the gas stream. Such coalescence of the molten metal droplets is promoted where the surface of the eliminating medium is of such a character as to be "wetted" by the molten metal particles. It is further possible that 20 the molten metal droplets, with little or no coalescence, are mechanically entrapped in the eliminating medium due to the tortuous passages therein, and thereby removed from the gaseous product. Whatever the true explanation may be, the facts remain that 25 under the conditions of operation herein described the gaseous product is very substantially freed of contaminating metals and that the contaminating metals removed from 30 the gaseous product remain with the eliminating medium in a form less readily returned to the gaseous product than the form in which these metals exist in the zinciferous material of the smelting charge.
- 35 Coalescence of the minute molten particles or droplets of the contaminating metals can be promoted by maintaining the eliminating medium at a substantially lower temperature than the zinc smelting temperature, but preferably not so low as to condense any substantial amount of zinc vapor. In passing through the eliminating medium maintained at such lower temperatures, the concentration of the minute metal particles in a unit 45 volume of gas is increased, thereby increasing the possibilities of collision with one another and the formation of larger particles or droplets. Moreover, this higher concentration of the metal droplets in a unit 50 volume of gas results in more frequent and ready impingement of the droplets against the surfaces of the eliminating medium and thereby promotes the possibilities of coalescence and the more complete removal of the 55 contaminating metals from the gaseous product. It is, accordingly, our preferred practice to maintain the eliminating medium at a temperature intermediate the temperature at which zinc is reduced from its compounds 60 and the temperature at which metallic zinc vapor is condensed, and of course below the temperature at which lead (or other contaminating metal) will remain with the gaseous product, under the prevailing operating 65 conditions.

The desired temperature regulation and control of the eliminating medium may be effected in any appropriate and convenient manner. This may be conveniently done by surrounding the eliminating medium with means for varying or adjusting the heat radiation therefrom. We have secured excellent results in practice by confining the eliminating medium in a vertical tube several feet in length and surrounded by heat insulating material of variable thickness or effectiveness. By appropriately adjusting the effectiveness of the heat insulating material, the radiation of heat from the tube can be so controlled as to maintain the desired temperature of the eliminating medium.

We have found that the character and composition of the gaseous product resulting from the zinc smelting operation has an important bearing on the effectiveness of the removal of the lead and other contaminating metals in accordance with the principles of our invention. The best results are obtained when the gaseous product is a substantially continuous stream of zinc vapor and carbon monoxide relatively constant in volume and composition and practically free of oxidizing gases. Such a gaseous product may be advantageously obtained in the process of smelting an agglomerated or briquetted charge of zinciferous and reducing materials in accordance with the principles disclosed in the copending application of Messrs. Breyer and Bunce, Serial No. 163,902, filed January 27, 1927.

Where the process of the aforementioned Breyer and Bunce application is carried out in an upright or vertical retort, the improvements of the present invention may advantageously be embodied in the process by providing an upper prolongation of the retort, above the reducing zone therein, adapted to confine the eliminating medium which in this case will be composed of a body or column of the agglomerated zinc smelting charge itself about to be advanced or introduced into the smelting zone of the retort. The agglomerated charge as a whole then progressively passes through the vertical retort and its prolongation and is heated in the reducing zone of the retort to a sufficiently high temperature to reduce compounds of zinc and volatilize the resulting metallic zinc and in the prolongation of the retort is maintained at an appropriate temperature to prevent volatilization of lead compounds and to effect substantial removal of lead (and/or other contaminating metals) from the gaseous product of the reduction, preferably without condensing any substantial amount of zinc vapor. The eliminating medium is thus superposed on the zinc smelting charge undergoing reduction and, with appropriate renewal or introduction of fresh charge at the top, progressively descends from the elimi-

nating zone to the smelting zone, and the worked-off or exhausted agglomerates are appropriately withdrawn from the bottom of the retort. The de-leaded gaseous product is withdrawn from the prolongation at or near the top of the de-leading body of agglomerates and is conducted to the zinc recovery apparatus, such as a condenser for zinc metal. To prevent air or oxidizing gases being carried into the eliminating medium during the introduction of fresh charge, it is our preferred practice to introduce the charge at a temperature at which there is sufficient gas evolution from the fresh charge to prevent the entraining of air. Under these condition of operation, it is of course necessary to maintain the eliminating medium at a carefully regulated temperature below that of zinc reduction, in order to avoid reduction of the zinciferous material of the eliminating medium with the consequent decrease in the effectiveness of the medium for removing lead.

Practicing our present invention in the manner described in the preceding paragraph, with the eliminating medium maintained at a carefully regulated temperature of about 800 to 900° C., we have obtained zinc metal containing from 0.019 to 0.050% of lead from a zinc concentrate containing from 65-70% of zinc and 1.5 to 3.5% of lead. Following the same procedure, but omitting the deleading operations of the present invention, the resulting zinc metal contains from 0.5 to 1.25% lead. Likewise, working this same ore in an ordinary zinc distillation furnace in accordance with the customary spelter retort practice, the resulting zinc metal contains 1% lead and over.

Applying the principles of the invention to a zinc ore containing a relatively small amount of lead, smelted in accordance with the Breyer and Bunce method hereinbefore particularly described, we have succeeded in producing zinc metal containing from 0.0024 to 0.0032% lead. Treating this same ore by the same procedure, but omitting the features of the present invention, the resulting zinc metal contains from 0.08 to 0.12% lead. Likewise, in treating this same ore in accordance with the present spelter retort practice the resulting zinc metal contains from 0.08 to 0.12% lead.

The practice of the invention correspondingly lowers the percentages of other contaminating metals present in the resulting zinc metal, as compared with the percentages of these metals that are found in zinc metal produced by the heretofore customary or known methods of zinc smelting. Thus, we have succeeded by the practice of the invention in reducing the percentages of such metals from readily determinable amounts to substantially negligible and practically indeterminable amounts.

Various forms of apparatus, other than those heretofore referred to, may be employed in practicing the invention. In any case the eliminating medium, appropriately confined or enclosed, is disposed intermediate the zinc-smelting chamber and the zinc recovery apparatus. The length of the eliminating medium, in the direction of gas flow, should be sufficiently long to effect substantially complete removal of lead from the gaseous product passing therethrough. Moreover, the eliminating medium should preferably be susceptible of convenient temperature control. While the eliminating medium may be periodically renewed, as its lead-removing capacity becomes lessened, it is our preferred practice to progressively move the eliminating medium through its enclosure, preferably in a direction opposite to that of the direction of flow of the gaseous product, and to renew the medium from time to time by fresh material added thereto at a temperature approximating the temperature at which the medium is maintained. Thus, vertically disposed cylindrical receptacles are especially suited for confining or enclosing the eliminating medium, since the heat radiation from such receptacles can be conveniently and accurately controlled, the eliminating medium can be conveniently renewed therein or progressively passed therethrough, and the gaseous product can be conveniently conducted thereto and withdrawn therefrom.

While it is our preferred practice to conduct the elimination of the contaminating metals without substantial condensation of metallic zinc vapor in the eliminating medium, this is not essential, since whatever zinc is condensed in the eliminating medium can be subsequently revolatilized and recovered. Such subsequent revolatilization and recovery of any condensed zinc is particularly simple where the eliminating medium is composed of one or more ingredients of the zinc smelting charge, since in such a case the material of the eliminating medium, after it has completed its role in the eliminating operation, may be introduced into the zinc smelting chamber where any condensed zinc is revolatilized and returned to the gaseous product. In such a case it is, of course, desirable that the transfer of the material from the eliminating operation to the smelting operation be effected with as little loss of heat as possible.

While we have hereinbefore particularly mentioned the recovery of the metallic zinc vapor from the deleaded gaseous product in the form of zinc metal or spelter, it is to be understood that the zinc vapor may be recovered in other forms of zinc products. Thus, the zinc vapor may be condensed as zinc dust, or may be oxidized and collected as zinc oxide. In any case, the practice of the invention enables the production of zinc products more nearly free from lead and similar contami-

nating metals than could otherwise be obtained by pyrometallurgical methods from the same zinciferous materials.

In the appended claims we intend the term 5 contaminating metal to cover any metal whose boiling temperature is above that of zinc but which accompanies the gaseous product of the zinc smelting operation and in particular lead, tin, antimony, bismuth, germanium and probably thallium, aluminum and magnesium.

We claim:

1. The improvement in the reduction of zinciferous material containing at least one 15 contaminating metal which comprises conducting the gaseous product of the reducing operation through a hot eliminating medium maintained under reducing conditions at a temperature sufficiently low to effect substantial 20 removal of said contaminating metal from said gaseous product, renewing said eliminating medium from time to time by fresh eliminating material added thereto at a temperature approximating that at which 25 the medium is maintained, and subjecting the thus-treated gaseous product to appropriate treatment for the recovery of the zinc content thereof.

2. The improvement in the reduction of 30 zinciferous material containing at least one contaminating metal which comprises conducting the gaseous product of the reducing operation through a hot eliminating medium maintained under reducing conditions at a 35 temperature sufficiently low to effect substantial removal of said contaminating metal from said gaseous product, progressively moving said eliminating medium in a direction opposite to the direction of flow of the 40 gaseous product therethrough, renewing said eliminating medium from time to time by fresh eliminating material added thereto at a temperature approximately that at which the medium is maintained, and subjecting the 45 thus-treated gaseous product to appropriate treatment for the recovery of the zinc content thereof.

3. The improvement in the reduction of 50 zinciferous material containing at least one contaminating metal which comprises conducting the gaseous product of the reducing operation through an eliminating medium which will withstand the prevailing temperature and not react with or contaminate 55 metallic zinc vapor so as to effect the subsequent recovery of zinc, progressively moving said eliminating medium through the path of flow of the gaseous product, and subjecting the gaseous product thus substantially freed of said eliminating metal to appropriate treatment for the recovery of the zinc content thereof.

4. The improvement in the reduction of 60 an agglomerated charge of mixed zinciferous material and carbonaceous reducing agent

containing at least one contaminating metal which comprises progressively passing the agglomerated charge through a reduction chamber, conducting the gaseous product of the reducing operation through an 70 eliminating medium which will withstand the prevailing temperature and not react with or contaminate metallic zinc vapor so as to effect the subsequent recovery of zinc, progressively passing said eliminating 75 medium through the path of flow of the gaseous product, and subjecting the gaseous product thus substantially freed of said contaminating metal to appropriate treatment for the recovery of the zinc content thereof. 80

5. The method of reducing zinciferous material containing tin in objectionable amount which comprises conducting a substantially continuous stream of the gaseous product of the reducing operation through a hot eliminating medium maintained under reducing conditions and which will withstand the prevailing temperature and not react with or contaminate metallic zinc vapor so as to effect the subsequent recovery of zinc, maintaining 90 said eliminating medium at a temperature adapted to effect substantial removal of tin from said gaseous product without condensing any substantial amount of zinc vapor, progressively moving said eliminating medium through the path of flow of the gaseous product, and subjecting the gaseous product thus substantially freed of said tin to appropriate treatment for the recovery of the zinc content thereof. 95

6. The improvement in the reduction of zinciferous material containing at least one contaminating metal which comprises conducting the gaseous product of the reducing operation through a hot eliminating medium removed from and kept out of contact with the reducing operation, said eliminating medium being maintained under reducing conditions and which will withstand the prevailing temperature and not react with or contaminate metallic zinc vapor so as to effect the subsequent recovery of zinc, maintaining 100 said eliminating medium at a temperature adapted to effect substantial removal of said contaminating metal from said gaseous product without condensing any substantial amount of zinc vapor, progressively moving said eliminating medium through the path of flow of the gaseous product, and subjecting the gaseous product thus substantially freed of said contaminating metal to appropriate treatment for the recovery of the zinc content thereof. 105

7. The improvement in the reduction of zinciferous material containing at least one 110 contaminating metal which comprises conducting the gaseous product of the reducing operation through a hot eliminating medium removed from and kept out of contact with the reducing operation, said eliminating medium being maintained under reducing conditions and which will withstand the prevailing temperature and not react with or contaminate metallic zinc vapor so as to effect the subsequent recovery of zinc, maintaining said eliminating medium at a temperature adapted to effect substantial removal of said contaminating metal from said gaseous product without condensing any substantial amount of zinc vapor, progressively moving said eliminating medium through the path of flow of the gaseous product, and subjecting the gaseous product thus substantially freed of said contaminating metal to appropriate treatment for the recovery of the zinc content thereof. 115

8. The improvement in the reduction of zinciferous material containing at least one 120 contaminating metal which comprises conducting the gaseous product of the reducing operation through a hot eliminating medium maintained under reducing conditions at a temperature sufficiently low to effect substantial 125 removal of said contaminating metal from said gaseous product without condensing any substantial amount of zinc vapor, progressively moving said eliminating medium through the path of flow of the gaseous product, and subjecting the gaseous product thus substantially freed of said contaminating metal to appropriate treatment for the recovery of the zinc content thereof. 130

tial removal of said contaminating metal from said gaseous product, renewing said eliminating medium by progressively moving the medium and adding fresh eliminating material thereto at a temperature approximating that at which the medium is maintained, and subjecting the gaseous product thus substantially freed of said contaminating metal to appropriate treatment for the recovery of the zinc content thereof.

8. The improvement in the reduction of zinciferous material containing at least one contaminating metal which comprises conducting a substantially continuous stream of the gaseous product of the reducing operation through a substantially uniformly porous eliminating medium composed of a material which will withstand the prevailing temperature and not react with zinc, maintaining said eliminating medium at an elevated temperature sufficiently low to effect substantial removal of said contaminating metal from said gaseous product without condensing any substantial amount of zinc vapor, renewing said eliminating medium from time to time by fresh eliminating material added thereto at a temperature approximating that at which the medium is maintained, and appropriately recovering the zinc content of the thus-treated gaseous product.

9. The improvement in the reduction of zinciferous material containing at least one contaminating metal which comprises conducting a substantially continuous stream of the gaseous product of the reducing operation through a substantially uniformly porous eliminating medium composed of a material which will withstand the prevailing temperature and not react with zinc, maintaining said eliminating medium at an elevated temperature sufficiently low to effect substantial removal of said contaminating metal from said gaseous product without condensing any substantial amount of zinc vapor, renewing said eliminating medium by progressively moving the medium and adding fresh eliminating material thereto at a temperature approximating that at which the medium is maintained, and appropriately recovering the zinc content of the thus-treated gaseous product.

10. The improvement in the reduction of zinciferous material containing at least one contaminating metal which comprises conducting a substantially continuous stream of the gaseous product of the reducing operation through a substantially uniformly porous eliminating medium composed of a material which will withstand the prevailing temperature and not react with zinc, progressively moving said eliminating medium in a direction opposite to the direction of flow of the gaseous product therethrough, renewing said eliminating medium from time to time by fresh eliminating material added thereto at a temperature approximating that at which

the medium is maintained, and subjecting the gaseous product thus substantially freed of said contaminating metal to appropriate treatment for the recovery of the zinc content thereof.

In testimony whereof we affix our signatures.

EARL H. BUNCE.  
GEORGE T. MAHLER.

70

75

80

85

90

95

100

105

110

115

120

125

130